

## UNITED STATES PATENT OFFICE

2,095,574

## MINING FUSE

Maurice Roumazeilles, Joinville le Pont, and Roger Harlé, Pitres, France, assignors to Societe dite Harlé Frères & Co., S. A. R. L., Pitres (Eure), France

No Drawing. Application May 4, 1936, Serial No. 77,878. In France May 10, 1935

9 Claims. (Cl. 102—8)

The present invention relates to mining fuses and especially mining fuses for firing liquid oxygen cartridges.

The fuses that are employed at the present time for firing liquid oxygen cartridges have the drawback that they do not prevent the formation of external sparks which, in the presence of the oxygen stream, considerably accelerate the rate of combustion and therefore endanger the life 10 of the person that is making use of them.

It has been endeavoured to obviate this drawback by impregnating these fuses with saline solutions, or, in a more general manner, impregnating masses the decomposition of which, under 15 the effect of the heat resulting from the combustion of the black powder core and from the external sparks, produces either the formation of a protective and extinguishing gaseous layer or the vitrification of the impregnating mass, giving the 20 same result.

It was also suggested to make fireproof compositions of matter, especially for the manufacture of insulating materials for use in other branches of the art, for instance for making electrical 25 conductors. These compositions consist of mixtures of polysulphides of olefines of rubber and of fillers. They may also consist of the following matters:

Resins plastified by a tricresylphosphate; 30 Gutta-percha mixed with rubber and resin;

Hydrocarbons mixed with rubber and a halogenous naphthalene;

Rubber mixtures containing aliphatic polymeric compounds having a high percentage of 35 chlorine and aromatic chlorinated hydrocarbons.

But these compositions of matter do not possess the properties above stated necessary for making mining fuses more especially intended for firing liquid oxygen cartridges.

The object of the present invention is to provide a mining fuse which avoids all the drawbacks above mentioned.

To this effect, the present invention contemplates the coating of a mining fuse having a 45 combustible core of the usual type with a thin, flexible and non-viscous coating or shell composed of a chloronaphthalene, having a high percentage of chlorine, with the admixture of chlorinated rubber, this latter ingredient representing less than 30% (preferably in the neighborhood of 12%) by weight of the mixture, and acting as a plastifier for and at the same time fireproofing the coating.

If desired, additional plastifying substances 50 may be added to this mixture, such as for exam-

ple, tricresyl- and triphenylphosphates with or without the admixture of a filler such as, preferably, lamp black. In order to prevent the fuse from adhering while being wound about itself, it may be covered with a layer of powdered mica, 5 which is preferably applied immediately after being coated and while the coating is still in a wet state. The mixture thus formed is perfectly stable and neutral at temperatures below 150° C., and it is especially suited for application upon 10 the fuse at lower temperatures more compatible with the prevention of deterioration of the powder comprising the combustible core of the fuse (below 105° C.). Another important property of the novel coating is that it may be applied in very thin layers to the fuse at these 15 preferred temperatures.

When brought to temperatures above 150° C. by the heat given off by the combustion of the fuse, the mixture comprising the coating will 20 form a shell which normally is incombustible, and, while melting, will gradually coat the fuse as the normal combustion of the latter proceeds.

Thus, the coating provided in accordance with the present invention possesses the following desirable properties. In the heated state, it is liquid at the preferred temperatures of application, or otherwise the powder core would be deteriorated, and it is sufficiently liquid to coat an ordinary fuse with a very thin uniform shell at a 25 very rapid speed. In the cold state, the coating is adherent to the fuse base, flexible, and hard enough at normal temperatures to prevent sticking to itself when wound, or to other substances with which it may come in contact. The covering is also very homogeneous, stable, impermeable, and insoluble.

One specific example of the reduction of the present invention to practice is as follows: 4500 gr. of tetrachloronaphthalene are melted at a 40 temperature of approximately 120°, that is, somewhat above its melting point; 400 gr. of tricresylphosphate, such as ammonium tricresylphosphate, are then added; then there is added with constant stirring 600 gr. of chlorinated rubber; 45 and about 200 gr. of lamp black or any other suitable filling material may be added to the mixture. When thoroughly mixed the product may be applied directly to the fuse base,—which is preferably already tarred as in the usual case,— 50 by immersion of the fuse in the vessel containing the molten coating material.

It should also be noted that the mixture above indicated can be utilized in combination with pitches, tars, resins, plastic matter and the like. 55

In a general manner, while we have, in the above description, disclosed what we deem to be an efficient embodiment of the present invention, it should be well understood that we do not wish to be limited thereto as there might be changes made therein without departing from the principle of the present invention as comprehended within the scope of the appended claims.

What we claim is:

- 10 1. A safety fuse particularly adapted for use in connection with the firing of liquid oxygen cartridges in mining operations or the like, comprising a fuse having a combustible core and having a thin, flexible, non-viscous coating thereon composed of a mixture of tetrachloronaphthalene and chlorinated rubber, the latter ingredient not exceeding 30% by weight of the total mass of said mixture.
- 15 2. A safety fuse particularly adapted for use in connection with the firing of liquid oxygen cartridges in mining operations or the like, comprising a fuse having a combustible core and having a thin, flexible, non-viscous coating thereon composed of a mixture of tetrachloronaphthalene and chlorinated rubber, the latter ingredient comprising approximately 12% by weight of the total mass of said mixture.
- 20 3. A safety fuse particularly adapted for use in connection with the firing of liquid oxygen cartridges in mining operations or the like, comprising a fuse having a combustible core and having a thin, flexible, non-viscous coating thereon composed of a mixture of not under 70% by weight of tetrachloronaphthalene and not over 30% by weight of chlorinated rubber; together with an additional plastifier consisting of one selected from the following group:—tricresylphosphates and triphenylphosphates.
- 25 4. A safety fuse particularly adapted for use in connection with the firing of liquid oxygen cartridges in mining operations or the like, comprising a fuse having a combustible core and having a thin, flexible, non-viscous coating thereon composed of a mixture of not under 70% by weight of tetrachloronaphthalene and not over 30% by weight of chlorinated rubber; together with an additional plastifier consisting of ammonium tricresylphosphate.
- 30 5. A safety fuse particularly adapted for use in connection with the firing of liquid oxygen cartridges in mining operations or the like, comprising a fuse having a combustible core and having a thin, flexible, non-viscous coating thereon composed of a mixture of not under 70% by weight of tetrachloronaphthalene and not over 30% by weight of chlorinated rubber; together with a

filler and an additional plastifier consisting of one selected from the following group:—tricresylphosphates and triphenylphosphates.

6. A safety fuse particularly adapted for use in connection with the firing of liquid oxygen cartridges in mining operations or the like, comprising a fuse, having a combustible core and having a thin, flexible, non-viscous coating thereon composed of a mixture of not under 70% by weight of tetrachloronaphthalene and not over 30% by weight of chlorinated rubber; together with a filler consisting of lamp black and an additional plastifier consisting of one selected from the following group:—tricresylphosphates and triphenylphosphates.

7. A safety fuse particularly adapted for use in connection with the firing of liquid oxygen cartridges in mining operations or the like, comprising a fuse having a combustible core and having a thin, flexible, non-viscous coating thereon composed of a mixture of not under 70% by weight of tetrachloronaphthalene and not over 30% by weight of chlorinated rubber; together with an additional plastifier consisting of a tricresylphosphate; and an outer adhering layer of powdered mica.

8. A safety fuse particularly adapted for use in connection with the firing of liquid oxygen cartridges in mining operations or the like, comprising a fuse having a combustible core and having a thin, flexible, non-viscous coating thereon composed of a mixture of the following ingredients in the proportions substantially as set forth:—

|                        | Parts |
|------------------------|-------|
| Tetrachloronaphthalene | 45    |
| Chlorinated rubber     | 6     |
| A tricresylphosphate   | 4     |
| A filler               | 2     |

9. A safety fuse particularly adapted for use in connection with the firing of liquid oxygen cartridges in mining operations or the like, comprising a fuse having a combustible core and having a thin, flexible, non-viscous coating thereon composed of a mixture of the following ingredients in the proportions substantially as set forth:—

|                             | Parts |
|-----------------------------|-------|
| Tetrachloronaphthalene      | 45    |
| Chlorinated rubber          | 6     |
| Ammonium tricresylphosphate | 4     |
| Lamp black                  | 2     |

ROUMAZEILLES.

ROGER HARLE.